

Patented Sept. 2, 1941

2,254,777

# UNITED STATES PATENT OFFICE

2,254,777

## PROCESS OF PRODUCING ARTIFICIAL STAPLE FIBERS RESEMBLING WOOL

Paul Esseleman, Wolfen, Kreis Bitterfeld, and Fritz Davidshöfer, Dessau, Anhalt, Germany, assignors, by mesne assignments, to Walther H. Duisberg, New York, N. Y.

No Drawing. Application July 24, 1937, Serial No. 155,576. In Germany August 26, 1936

5 Claims. (Cl. 18—54)

Our present invention relates to a process of spinning artificial fibers from viscose solutions.

It is an object of the present invention to provide a process by which artificial staple fibers resembling wool are produced.

Further objects will be apparent from the detailed specification following hereafter.

According to this invention artificial fibers having an appreciably better resemblance to wool are obtained by spinning a more strongly ripened viscose directly into an alcoholic precipitating bath, for example into methanol, ethyl alcohol or the like, and then subjecting the freshly coagulated fibers to a final decomposition. The most satisfactory results in respect of curliness and power of adhesion are obtained if the fibers are cut into staple lengths before the decomposition, since the fibers can then shrink more completely. Obviously, however, the fiber can also be subjected to decomposition and finished in its endless uncut state. The final fixing of the fibers in the form of regenerated cellulose can be brought about in various ways, for example by treatment with hot air, whereby at the same time the alcohol associated with the fiber is evaporated and can be recovered, or by treatment with a hot acid or a hot salt solution.

The finished, after-treated and dried fibers have the appearance of wool in respect of curliness and superficial structure. Their physical properties can be regulated by stretching them during spinning, for example after they have left the first precipitating bath or during the first decomposition of the xanthate. The process may be conducted with the usual spinning nozzles having orifices of 0.07—0.09 mm. diameter or with nozzles having orifices of 0.5—0.8 mm. diameter and more; in the latter case the fiber may be simultaneously drawn out in a stretch-spinning funnel.

The fibers may be desulfurized during coagulation or during the final decomposition.

Instead of methanol or ethanol any mono- or polyvalent alcohols or mixtures of alcohols may be used. There may be used mixtures of alcohol and water, but the water content of these mixtures should not exceed 30 per cent.

The temperature of the final decomposition may be from about 90 to 150° C., in some cases even higher.

The following example illustrates the invention:

Viscose having a content of cellulose of 8 per cent and a content of alkali of 8 per cent is ripened to a salt point of 0.5 and then spun in a solution composed of 90 per cent of methanol and 10 per cent of water. The freshly coagulated fibers are then cut into staple lengths and decomposed by means of a hot salt solution having

a temperature of 103° C. The fibers are then washed, after-treated and dried. The fibers thus obtained have a wool-like appearance and, although they have been spun from cellulose, a fine matt luster. Particularly striking is its good curliness with very finely curved crimps. Under the microscope the fiber exhibits numerous crater-like openings which impart to it a high capacity of adhesion. The fibers have a round cross-section.

What we claim is:

1. A process of producing artificial staple fibers resembling wool, which comprises spinning viscose in a precipitating bath containing more than 15 70 per cent of an alcohol of comparatively low boiling point and subsequently decomposing the freshly coagulated xanthate threads by subjecting said threads to the action of a medium having a temperature of from about 90 to about 150° C.

2. A process of producing artificial staple fibers resembling wool, which comprises spinning viscose in a precipitating bath containing more than 15 70 per cent of an alcohol of comparatively low boiling point, cutting the freshly coagulated 20 xanthate threads into staples and subsequently decomposing said threads by subjecting them to the action of a medium having a temperature of from about 90 to about 150° C.

3. A process of producing artificial staple fibers resembling wool, which comprises spinning viscose in a precipitating bath containing more than 30 70 per cent of an alcohol of comparatively low boiling point, cutting the freshly coagulated 35 xanthate threads into staples and subsequently decomposing said threads by subjecting them to the action of a hot acid solution having a temperature of from about 90 to about 120° C.

4. A process of producing artificial staple fibers 40 resembling wool, which comprises spinning viscose in a precipitating bath containing more than 70 per cent of an alcohol of comparatively low boiling point, cutting the freshly coagulated xanthate threads into staples and subsequently 45 decomposing said threads by subjecting them to the action of a hot inorganic salt solution having a temperature of from about 90 to about 130° C.

5. A process of producing artificial staple fibers resembling wool, which comprises spinning viscose containing 50 8 per cent cellulose and 8 per cent alkali and having a salting point of 0.5 in a precipitating bath comprising 90 per cent methanol and 10 per cent of water, cutting the freshly coagulated xanthate threads into staples and decomposing said threads by means of a hot salt solution having a temperature of about 103°.

PAUL ESSELMANN.  
FRITZ DAVIDSHÖFER.